

Aug. 29, 1933.

E. CADGÈNE

1,924,677

FABRIC AND METHOD OF TREATING THE SAME

Filed June 23, 1931

FIG. 1.



FIG. 2.



FIG. 3.



FIG. 4.



INVENTOR  
ERNEST CADGÈNE

BY  
Richard A. Seier  
ATTORNEYS

## UNITED STATES PATENT OFFICE

1,924,677

## FABRIC AND METHOD OF TREATING THE SAME

Ernest Cadgène, Englewood Cliffs, N. J.

Application June 23, 1931. Serial No. 546,369

2 Claims. (Cl. 41—41)

This invention relates to improvements in textile fabrics and the method of treating the same.

An object of the invention is to produce a fabric which will simulate embroidery in appearance, particularly eyelet embroidery, the desired effect being accomplished by the deposition of a decorative substance applied to said fabric contiguous to a portion or portions thereof from which fibers comprising the fabric have been removed.

Another object resides in the formation of an opening or eyelet in a fabric and the implanting of a decorative substance thereon around the edge of said opening so as to bind the fibers and thereby prevent fraying of the fabric.

The above and other objects will appear more clearly from the following detailed description, when taken in connection with the accompanying drawing, which illustrates preferred embodiments of the inventive idea.

In the drawing—

Figure 1 is a plan view illustrating one form of fabric made in accordance with the invention;

Figure 2 is a section on the line 2—2 of Figure 1;

Figure 3 is a plan view of another form; and

Figure 4 is a similar view, partly broken away, of still another form.

The terms "eyelet" and "opening" as used in the description and claims are employed to designate an opening where all the material is removed, as shown in Figures 1 and 2, or where only part of the material is removed or changed, as in Figures 3 and 4. The eyelets may be of any desired size or form.

In its general aspects the invention contemplates a fabric the appearance of which closely resembles that of eyelet embroidery work and, in order to accomplish the decorative effect of such work, it is proposed to remove portions of the fibers constituting the fabric to simulate the eyelets of the embroidery, the bas-relief ornamentation of said embroidery being obtained by applying a decorative composition of any nature to the fabric in close proximity to the parts thereof from which the fibers have been removed. The two steps of removing the fibers and applying the decorative substance may be accomplished in either order of succession.

In Figure 1 there is shown a fabric 5 made from any suitable fiber, such as cotton, silk, wool, rayon and the like, and provided with openings 6 of desired configuration which, in combination with any suitable composition 7 applied around

the edges of said openings, comprise a composite bas-relief ornamentation. The composition 7 is of such nature that, when implanted on the fabric contiguous to the edges of the openings, it will bind the loose ends of the fibers forming said edges and thus prevent fraying of the material. The openings 6 of the present embodiment may be formed by removing the fibers either through the use of some well-known mechanical means, such as a punch, or by employing an equally well-known chemical destroying agent suitable to the particular kind of fiber used in weaving the fabric. Any known means of applying the chemical destroying agent may be employed, such as screens or stencils, or by running the fabric over an engraved roller. The effect of the application of the destroying agent to the fabric is to produce carbonization of the fibers which come in contact therewith after the fabric has been dried and heated, following which said fabric may be brushed or washed to remove said fibers.

The step of depositing the composition 7 on the fabric involves its application thereto in registry with the portions which have come in contact with the destroying agent, or the edges of the openings that have been formed by mechanical means; or, conversely, if the composition is applied before the destroying agent as previously suggested, said agent is imprinted on the fabric in registration with the ornamentation produced by said composition so that only the fibers surrounded by the latter will be destroyed. Any one of several known methods of securing registration of the two components of the design may be used, such as the one shown in United States Letters Patent No. 1,673,934, issued June 19, 1928, wherein registry of color and flock printing patterns are obtained by the use of a stencil which deposits the flock material on the fabric that has been previously printed with a color pattern. Thus, in the present method, after the application of the destroying agent to the fabric, or the formation of the openings therein, said fabric can be run through the machine shown in said patent to obtain the deposit thereon of the composition 7 in registry with the portions affected by said agent, or with said openings.

The composition 7 may be composed of a glue, cellulose, or albumen solution, or may be a plastic substance such as used in the well-known flock printing process of the prior art. The latter substance is the one referred to in the above-mentioned patent and is readily adapted for use in the present method. It is of such a character

that when deposited upon the fabric it permeates the interstices thereof and being of a sticky nature permits of the application thereto, before drying, of other decorative substances, such as metal powders and short fibers of other material, thereby creating a wide range for the production of ornamental effects. Having the quality of adhesion also enables said substance to permanently attach itself to the fabric and securely bind together the fibers thereof and, when dried, forms a bas-relief ornamentation which will closely simulate eyelet embroidery.

After the application of said substance, the fabric is thoroughly dried and during this process said substance hardens so that it becomes permanently affixed to the fabric and constitutes a binder which prevents fraying of the material around the eyelets. When a destroying agent is used to outline the openings 6, the fibers affected thereby carbonize during the drying and heating process and at the conclusion thereof are removed by washing or brushing the fabric.

As a specific example, a length of cotton fabric may be passed over an engraved roller coated 25 with a fiber-destroying agent consisting of a gum solution containing about 375 grams per liter of aluminum chloride. This solution acts to produce the desired pattern of eyelets or openings. The fabric is then passed through a machine such as shown in the above-mentioned Letters Patent wherein, by means of a stencil, a coating of varnish of suitable thickness is applied to the fabric in registry with the portions thereof previously treated with the destroying 30 agent. While this varnish is still wet a powder of any color, which may be made from metal or very short fibers of cotton, silk, wool, or rayon, is deposited upon the fabric. This powder adheres to the parts of the fabric which are coated with the varnish and the remainder is shaken off, leaving the desired pattern of flock on the fabric. The material so treated is dried, heated and then brushed or washed to remove the fibers which have been affected by the destroying agent. The 40 result is a cotton fabric with imitation eyelet embroidery in which the flock composition constitutes a binder about the edges of the eyelets or openings to prevent fraying of the material.

When using a fabric made of animal fibers, 50 such as pure silk or wool, or mixtures thereof, the fiber-destroying agent employed may be a gum solution containing about 500 grams per liter of caustic soda of a strength of 32° Baumé. The remainder of the treatment of the fabric is the same as described in the above example.

Another method of attaining the desired effect is illustrated in Figure 3. In this example, the fabric 8 is woven with at least two fibers of different characteristics, one of which is capable of

resisting the carbonizing effect of an agent employed to destroy the other. Thus, fibers of a vegetable nature, such as cotton, may be combined with natural silk, acetate of cellulose, and wool fibers, and, if it is desired to remove the cotton fibers in certain portions of the fabric, a destroying agent, for example sulphuric acid or a solution of aluminum chloride may be used; or, if the other fiber is to be destroyed, it may be treated with an alkali solution. It will be appreciated, of course, that many other combinations of fibers may be employed, an important feature being that at least one of the fibers is modified.

The result of the foregoing treatment is the formation of an opening 9 in the fabric across which extends the undestroyed fibers 10 which give an openwork or mesh effect instead of the unobstructed eyelet shown in Figures 1 and 2. The ornamentation of the fabric by the application of the composition 11, similar to the material 7, proceeds in the same manner as previously described.

In Figure 4 an effect is shown which is practically the same as that illustrated in Figure 3, but in this instance two separate fabrics 12 and 13 of different characteristics are used instead of the single fabric comprising the interwoven contrasting fibers. The two fabrics 12 and 13 may be superimposed and secured together by a suitable adhesive preliminary to the treatment with the destroying agent which forms the openings 14 and leaves the undestroyed fibers 15 of one of the fabrics extending across said openings. Again, a composition 16 like that previously described is deposited upon one of the fabrics in registry with the openings 14 and the nature of said composition is such that it will pass through the interstices of said fabrics in the manner indicated in Figure 2, and, upon drying, will act as a binder to firmly secure the fabrics together.

What is claimed is:

1. As a new article of manufacture, a textile fabric in which fibers forming a portion thereof are removed, a decorative composition implanted on said fabric around said portion and combining therewith to simulate embroidery, and another fabric of a different characteristic from the first-named fabric secured thereto in registry with said portion.

2. The method which comprises superimposing two fabrics of different characteristics, binding said fabrics together with a material which will pass through the interstices thereof, and applying a fiber-destroying agent contiguous to said material which will affect the fibers of only one of said fabrics.

ERNEST CADGENE.

135

60

65

70

75

80

85

90

95

100

105

110

115

120

125

130

135

140

145

150